

June 4, 1957

P. F. WINTERNITZ

2,794,316

OPERATING INTERNAL COMBUSTION BURNERS OF THE JET MOTOR TYPE

Filed Feb. 23, 1949



INVENTOR  
PAUL F. WINTERNITZ  
BY  
*D. Harrison*  
ATTORNEY

2,794,316

## OPERATING INTERNAL COMBUSTION BURNERS OF THE JET MOTOR TYPE

Paul F. Winternitz, New York, N. Y., assignor to Reaction Motors, Inc., a corporation of New Jersey

Application February 23, 1949, Serial No. 77,733

2 Claims. (Cl. 60—35.6)

This invention relates to a novel internal combustion burner of the jet motor type and to a novel method of operating such a burner to prevent burn-out of the combustion chamber.

Jet motors have become of increasingly great importance in recent years. One of the difficulties facing the designers of such motors has been the tendency of their internal combustion chambers to burn out due to erosion and the high temperature of operation.

One object of the present invention is to provide a novel internal combustion burner of the jet motor type which is protected against premature burn-out. Another object is to provide a novel method for operating such a burner so that burn-out of the combustion chamber is prevented and the life of the motor is substantially extended.

The single figure of the drawing is a schematic, longitudinal, mid-sectional view of a jet motor which can be operated by the method of the invention.

In accordance with the present invention an internal combustion chamber is protected from burn-out by coating its inside surface with a refractory material which increases the life of the burner.

It has been observed that when the refractory coating is applied before operation of the burner it is effective for only a relatively short time and then substantially disappears from the chamber wall. This may be due to erosion, to vaporization of the coating due to the high temperature of the operation, and also to differential expansion between the chamber wall and the coating when a jet motor is started or stopped and a substantial temperature change takes place. To overcome this difficulty, therefore, it is preferred to build up and maintain or renew the coating endogenously during operation of the combustion chamber. This is accomplished by continuously and concurrently injecting into the chamber an oxidant, such as liquid or gaseous oxygen, ozone, or peroxides, and a fluid fuel comprising a substance which burns in the oxidant to form a refractory solid material which is continuously deposited and built up or renewed on the internal wall of the chamber to maintain a protective coating thereon. The fluid fuel advantageously can comprise readily combustible organic and inorganic silicon compounds which burn in oxygen to form a refractory deposit of silica. Examples of such compounds are tetra ethyl orthosilicate, tetra methyl orthosilicate, trichlorosilane, dichlorosilane, and other combustible halogenated silanes or esters of orthosilicic acid or of their derivatives. A glassy protective coating of boron oxide is formed when the fluid fuel comprises diborane. A protective coating of aluminum oxide is obtained when the fuel comprises powdered aluminum.

In one specific example of how the method of the invention was performed, a water-cooled jet motor B was operated on a test block by introducing monomeric tetra ethyl orthosilicate through a supply conduit 11 to a header 13, from which it was discharged into an internal combustion chamber 15 through a plurality of injector

nozzles 17 arranged in a ring at one end of the chamber. At the same time oxygen was introduced through a supply conduit 19 and injected centrally into chamber 15 through an injector nozzle 21 arranged centrally within the ring of nozzles 17. At an oxygen-to-fuel ratio of .904 the motor was operated for several runs which lasted between 18.4 and 42 seconds, and in each run a protective coating 23 of silica was built up and maintained on the previously uncoated wall 25 of the combustion chamber, including the throat section 27. Motors having combustion chamber walls of both stainless steel and of graphite were operated in this way.

In a second series of tests a fuel consisting of high octane gasoline containing 30% of aluminum powder suspended therein was injected through the nozzles 17 while oxygen was injected through the nozzle 21. Upon conclusion of each run it was found that the previously uncoated wall 25 of the combustion chamber, including the throat 27, was coated with a protective layer 23 of aluminum oxide.

A third series of tests was made using diborane as the fuel. Runs were made with the diborane injected through the annularly arranged nozzles 17 and oxygen injected centrally through nozzle 21; and other runs were made with the diborane injected centrally through the nozzle 21 and the oxygen through the annularly arranged nozzles 17. With both arrangements a glassy refractory coating 23 of boron oxide was built up and maintained on the previously uncoated wall 25 of the combustion chamber, including the throat 27. However, it was observed that with diborane injected centrally the coating was practically all boron oxide, whereas with the reverse arrangement some free boron was present in the coating.

While specific embodiments of the novel method and apparatus have been described herein, for illustrating the principles of the invention, it is evident that changes in the method and apparatus can be made by persons skilled in the art, within the scope of the invention.

What is claimed is:

- 40 1. A method of operating and protecting from burn-out an internal combustion burner of the jet motor type having a combustion chamber with internal walls including a convergent portion adjacent a discharge outlet subject to the erosive action of high temperature fast moving combustion products which method comprises externally cooling such internal walls with a coolant; continuously and concurrently injecting into said combustion chamber under pressure an oxidant and a fluid fuel comprising at least in part a substance which burns in such oxidant 45 to form a refractory solid oxidation product; burning such fuel in said chamber at high temperature so that the gaseous combustion products are rapidly ejected from the combustion chamber between the convergent walls; and concurrently depositing, renewing and building up on 50 said internal walls including the convergent portion a protective coating comprising portions of said refractory solid oxidation product, the amount of such substance in the fuel being at least sufficient to provide deposition at a rate to maintain and renew the protective coating 55 on such internal walls and counteract said erosive action, said fluid fuel comprising a monomeric lower tetra alkyl orthosilicate.

- 60 2. A method of operating and protecting from burn-out an internal combustion burner of the jet motor type having a combustion chamber with internal walls including a convergent portion adjacent a discharge outlet subject to the erosive action of high temperature fast moving combustion products which method comprises externally cooling such internal walls with a coolant; continuously and concurrently injecting into said combustion chamber 65 under pressure an oxidant and a fluid fuel comprising at least in part a substance which burns in such oxidant to

form a refractory solid oxidation product; burning such fuel in said chamber at high temperature so that the gaseous combustion products are rapidly ejected from the combustion chamber between the convergent walls; and concurrently depositing, renewing and building up on said internal walls including the convergent portion a protective coating comprising portions of said refractory solid oxidation product, the amount of such substance in the fuel being at least sufficient to provide deposition at a rate to maintain and renew the protective coating on such internal walls and counteract said erosive action, said fluid fuel comprising monomeric tetra ethyl orthosilicate.

|              |                |                |
|--------------|----------------|----------------|
| 1,405,482    | Bostedo        | Feb. 7, 1922   |
| 1,888,749    | Urquhart       | Nov. 22, 1932  |
| 2,043,867    | Rava           | June 9, 1936   |
| 2,212,992    | Sowa           | Aug. 27, 1940  |
| 5 2,257,194  | Rosen          | Sept. 30, 1941 |
| 2,266,776    | Leum           | Dec. 23, 1941  |
| 2,268,589    | Heany          | Jan. 6, 1942   |
| 2,272,342    | Hyde           | Feb. 10, 1942  |
| 2,399,687    | McNabb         | May 7, 1946    |
| 10 2,432,109 | Zisman et al.  | Dec. 9, 1947   |
| 2,442,976    | Heany          | June 8, 1948   |
| 2,558,483    | Goddard        | June 26, 1951  |
| 2,563,305    | Britton et al. | Aug. 7, 1951   |

## References Cited in the file of this patent

## UNITED STATES PATENTS

15

1,167,135 Torsen ----- Jan. 4, 1916

445,506

## FOREIGN PATENTS

Great Britain ----- Apr. 14, 1936